

April 24, 1928.

1,667,408

R. S. ALLEN

## METHOD AND APPARATUS FOR COATING FABRICS

Filed Nov. 9, 1921

2 Sheets-Sheet 1

Fig. 2.



Fig. 3.



Fig. 1.



Inventor.  
Ralph S. Allen,  
C. Luther H. Braxton  
By his Attorney.

April 24, 1928.

1,667,408

R. S. ALLEN

METHOD AND APPARATUS FOR COATING FABRICS

Filed Nov. 9, 1921

2 Sheets-Sheet 2



Fig. 4



Fig. 5



Fig. 6

INVENTOR.  
RALPH S. ALLEN,

BY Chester W. Brasels  
ATTORNEY

## UNITED STATES PATENT OFFICE.

RALPH S. ALLEN, OF NEWARK, NEW JERSEY, ASSIGNOR TO DURATEX CORPORATION, OF NEWARK, NEW JERSEY, A CORPORATION OF NEW JERSEY.

## METHOD AND APPARATUS FOR COATING FABRICS.

Application filed November 8, 1921. Serial No. 513,908.

The present invention relates to coated fabrics and more particularly to a process and apparatus for applying coating compositions to fabrics.

- 5 In certain of the coated fabrics heretofore used the coating composition has been applied directly to the surface of a suitable fabric base without penetrating or saturating the warp and weft of the fabric. The 10 penetration and saturation of the fabric base are avoided because they tend to render the coated fabric stiff and inflexible and therefore unsuitable for the purposes to which coated fabrics are usually applied. In 15 coated fabrics formed in this manner the coating is held on the surface of the fabric principally by the adhesive strength between the coating and fabric at their contact surface, no substantial anchorage of the coating 20 in the fabric base being obtained owing to the difficulty of obtaining an anchorage without saturating the fabric base. The coating of coated fabrics of this character is therefore very weakly attached and has a strong tendency to peel from the fabric base if the fabric be bent or creased. Such fabrics are therefore not satisfactory for use as substitutes 25 for natural leather or other uses for which a flexible, durable fabric is required.
- 20 An object of the present invention is to provide a coated fabric in which the coating is tenaciously and flexibly anchored to the body of the fabric base.

Another object of the invention is to provide a coated fabric in which a substantial anchorage of the coating of the fabric base is obtained by means of anchoring portions of the coating composition extending from the under surface of the coating into the 40 body of the fabric.

A still further object of the invention is to provide a flexible coated fabric having a number of anchoring projections extending from the coating into the body of the fabric.

45 A further object of the present invention is to provide a method of coating fabrics in which a portion of the coating composition is drawn into the fabric base in such a manner as to form a number of anchorages connecting the coating to the body of the fabric base.

A still further object of the invention is to provide a method of coating fabrics in which a tenacious uniform anchorage of the 55 coating to the fabric base may be obtained.

A still further object of the invention is to provide an apparatus for coating fabrics by which a uniform and thorough anchorage of the coating in the fabric base may be obtained without soaking or saturating the 60 fabric base.

With these and other objects in view, the invention comprises the method and apparatus described in the following specification.

65 The various features of the invention are illustrated in the accompanying drawings in which,

Fig. 1 is a sectional elevation of a coating device embodying a preferred form of the 70 invention,

Fig. 2 is a sectional elevation of modified form of coating apparatus,

Fig. 3 is an elevation of a part of the coating apparatus shown in Fig. 2 taken at right 75 angles to the section of Fig. 2,

Fig. 4 is a cross section of a coated fabric showing in a diagrammatic manner a conventional embodiment of the invention,

Fig. 5 is a cross section on a greatly magnified scale of the invention as applied to the 80 common type of fabric base, and,

Fig. 6 is a cross section on a greatly magnified scale of a coated fabric embodying a 85 form of the invention as applied to a fabric base having a nap on the surface to which the coating is applied.

In the present invention the coating is attached or anchored to the fabric base by drawing a portion of the coating composition 90 into the fabric base to a sufficient extent to fill or partly fill the crevices and channels which may exist or may be formed in the body of the fabric base. In forming the coated fabric the coating composition is applied to one face of the fabric and a slight suction is applied to the opposite face of the fabric directly opposite the application of the coating sufficient to withdraw the air from the pores or channels of the fabric and draw thereinto a portion of the coating composition which thereupon fills or partly fills the crevices and channels and serves as an anchorage to attach the coating to the fabric base. To this end, the fabric to be coated 105 is drawn, under suitable tension, beneath a feed trough from which the coating composition is supplied to the upper face of the fabric through a narrow slot extending substantially the entire width of the fabric. 110

Immediately beneath the feed trough is positioned a suction or vacuum chamber having a slot or opening in its top wall immediately beneath the slot of the feed trough. 5 One side of the feed trough is preferably extended to such a distance, in relation to the vacuum chamber, as to form a doctor blade serving to regulate the thickness of the coating. As the fabric passes between 10 the feed trough and the vacuum chamber a layer of coating composition is applied to the nap and is immediately drawn into the fabric by the suction applied to the opposite side of the fabric. The width of the slot 15 in the vacuum chamber is of such a dimension as not to extend beyond the doctor blade and, as the fabric passes under the doctor blade, the effect of the vacuum therefore ends and any further tendency of the composition to saturate the fabric base is thereby avoided.

The fabric is thereupon drawn into a suitable drying or hardening chamber in which the coating is hardened or dried. If several 20 coatings are to be applied, the fabric may be passed beneath a number of feed troughs or successively beneath a single trough. In this case the suction or vacuum is used only in connection with the earlier coating which 25 penetrates into the fabric, the final coatings serving primarily to form a hard or finished surface on the softer body of the coating.

Any fabric suitable for use as a base for 30 coated fabrics and having a sufficiently open or porous texture to permit the coating composition to be drawn thereinto may be employed. A fabric base having a nap or pile raised on the side to be coated may be employed or a woven fabric having a felted or partly felted structure may also be employed. The degree of vacuum and the duration of 35 its time of application are so adjusted as to permit the formation of an anchorage without completely saturating or penetrating the fabric base.

Referring more particularly to the accompanying drawings, a sheet of fabric 10 is drawn from a suitable roll or source of supply, not shown, around a tension roll 12 and idler or positioning rolls 14 and 16 and is passed beneath a composition feed trough 18, in such a manner that the face to be coated is uppermost as the fabric passes under the 40 trough. The feed trough 18 is preferably formed of two sides, 20 and 22, which converge to a narrow slot 24 at their lower end. Positioned immediately beneath the feed trough 18 is a vacuum chamber, 26, which is 45 connected by a connecting pipe 28 with a suitable suction device or means for producing a partial vacuum, not shown. The upper surface of the suction or vacuum chamber 26 is provided with a longitudinal slot 30, which is directly beneath the slot 24 of

the feed trough, and which may be of a somewhat greater width than the slot 24. The side 22 of the trough 18 is extended downwardly to within a short distance of the upper surface of the suction chamber 70 26 and the lower edge serves as a doctor blade to regulate the thickness of the coating applied to the fabric. In Figs. 4, 5 and 6 of drawings, the thickness of the coating composition above the fabric is relatively thin 75 as compared with the total thickness of the fabric. As the fabric passes over the slot 30 the air contained in the upper portion of the fabric is drawn downwardly out of the fabric and the coating composition is thereby permitted to sink into the channels or openings of the fabric base from which the air has been withdrawn. The vacuum or suction through the slot 30 is so regulated as to avoid drawing the coating entirely 80 through and saturating the fabric base. As the fabric passes under the doctor blade 22, it moves out of contact with the suction chamber 26 and any tendency toward a further, slow penetration or soaking of the fabric base is thereby avoided. The fabric is thereupon drawn over an idler or positioning roller 32 to a suitable drying or hardening chamber, not shown. When the coating 85 is sufficiently dried or hardened the stiffness which may result in forming certain kinds of coated fabrics may be lessened or removed by boarding the fabric in somewhat the same manner as leather is rendered more 90 flexible.

The fabric formed in the manner described above will ordinarily comprise a continuous surface coating 31, Figs. 4, 5, and 6, overlying the fabric base and having a large number of projections or short tentacles 33 95 extending downwardly from the surface of contact of the coating fabric into the body of the fabric base in the manner shown generally in Fig. 4 of the drawings. When the coating is applied to a woven cotton twill fabric the main portion of the coating will lie over, and contact with, the upper surface of the fabric base in the usual manner, as shown in Fig. 5 of the drawings, and a number of projections 33 will extend downwardly under the woof threads 35 or vice versa and will partly or very nearly encircle and grasp portions of the threads.

The invention may also be applied to a fabric having a pile or nap formed on the surface to be coated. This pile or nap is preferably short or shortened to give an upstanding character to the threads of the pile or nap and permit penetration by the coating composition. The coating composition is 120 accordingly drawn downwardly through the nap or pile into the hollows and depressions formed in the upper surface of the fabric base, as shown, for example, in Fig. 6. It 125 will be understood that any suitable coating 130

composition may be employed but for the manufacture of artificial leather a cellulosic composition such as the usual composition of pyroxylin and castor oil with suitable sol-

5 vent or any other suitable solution of cellulose is employed. The portion of the coating composition extending into the fabric base is preferably somewhat softer and more flexible than the surface of the coating and 10 contains a larger proportion of castor oil in order to give the fabric the desired flexibility. A harder surface coating having a higher percentage of pyroxylin is finally applied to the surface of the coating to give 15 greater wearing qualities and a better finish.

In the form of the invention shown in Fig. 1, the fabric is drawn taut over the suction chamber 26, the regulation of the thickness of the coating being obtained by the distance 20 between the doctor blade 22 and the upper surface of the suction chamber. In the modification shown in Figs. 2 and 3, the fabric is drawn tightly upwardly under the doctor blade 22.

25 Means are also provided in the modification shown in Fig. 2 for swinging the suction chamber 26 out of position to permit the application of succeeding coatings, for which the use of suction is not required. For this 30 purpose a rotatable or swinging connection 34 is provided between the pipe 28 and the suction chamber 26, and the chamber 26 is connected to the rotatable connection by means of a short pipe 36. Through this arrangement the suction chamber may be positioned in operative relation to the feed trough as shown in full lines or out of position as indicated in dotted lines in the drawings. The chamber 26 and pipe 36 are 35 secured in operative or inoperative position by means of a tightening bolt 38.

In the embodiment of the invention illustrated in Fig. 1, means are provided for raising the vacuum chamber 26 and adjusting its 40 position relative to the trough 18 and doctor blade 22 and thereby controlling the thickness of the coatings. To this end, the vacuum, chamber 26 is carried on a frame 37 having downwardly extending projections 45 or arms 39 which are clamped against corresponding uprights 29 by means of bolts 40 passing through vertical slots 42 in the uprights 29. By moving the bolts upwardly or downwardly, the position of the vacuum chamber 26 may be changed to adjust the thickness of the coating applied to the fabric. The suction pipe 28 is also adjustably connected to the chamber 26 by means of a pipe 44, which telescopes into a larger pipe 46 50 connected to the suction pipe 28 and fixed in position by means of a set screw 48.

By means of the above invention a tenacious and flexible anchorage may be cheaply and easily provided between the fabric base 55 and the coating applied thereto. It will be

apparent that various types of coating compositions may be employed and that other methods of forming the anchorage than that described in detail above may be employed without departing from the broader features of the invention.

Having described the invention what is claimed as new is:

1. A method of forming coated fabrics, which comprises applying a coating composition to the nap of a napped fabric and drawing said composition into said nap by suction applied to the opposite side of said fabric.

2. A method of forming coated fabrics, which comprises forming a fabric having a surface of fibres extending outwardly from the face of the fabric for a comparatively short distance, applying suction to a limited portion of the face of said fabric opposite said projecting fibres and applying a coating composition to the fibrous face opposite said portion.

3. A method of forming coated fabrics which comprises applying a coating composition to the fibrous face of a fabric having short projecting fibres, applying sufficient suction to the opposite face of said fabric to draw said composition to the ground of said fabric and immediately thereafter relieving said suction.

4. A method of forming coated fabrics which comprises passing a fabric having fibres extending transversely of said fabric over a slot in such a manner as to expose said fibres, applying a coating composition to said nap directly opposite said slot, withdrawing air from said fabric through said slot and thereupon reducing said coating to a uniform thickness by the application of a pressure plate.

5. A method of coating fabrics having a short nap which comprises, applying a coating composition to said nap and withdrawing air through said fabric from said nap immediately beneath said composition until said composition has been drawn into said nap for a substantial distance.

6. A method of coating napped fabrics which comprises applying a coating composition to the nap of said fabric and withdrawing air through said fabric from the nap immediately beneath said composition until said composition has been drawn into said nap a substantial distance, while avoiding drawing said composition through said fabric.

7. An apparatus for coating fabrics which comprises a suction chamber, a slot in said suction chamber, a composition feeding means above said slot, means for drawing said fabric over said slot and beneath said composition feeding means and a doctor blade arranged immediately back of said composition feeding means.

8. An apparatus for coating fabrics which comprises a long suction chamber, a slot in the upper part of said chamber, a composition feeding trough above said slot and a doctor blade adjacent said trough. 25
9. An apparatus for coating fabrics which comprises a long suction chamber, a slot in the upper wall of said chamber a feed trough above said slot, a doctor blade adjacent said trough and means for drawing a fabric between said trough and slot transversely of said slot and under said doctor blade. 30
- 10 An apparatus for coating fabrics, which comprises a suction chamber, a slot in the upper wall of said chamber, a composition feeding trough above said slot, a doctor blade adjacent said trough and means for drawing a fabric between said trough and said slot transversely of said slot and a tension roll 35 arranged to maintain said fabric under tension.
11. An apparatus for coating fabrics which comprises, a suction chamber, a slot in the upper wall of said chamber, a com- 40
- position feeding trough above said slot, a doctor blade adjacent trough, means for drawing a fabric between said trough and said feed slot and means for changing the position of said chamber relative to said feed trough and said doctor blade. 35
12. A method of forming coated fabrics which comprises applying a coating composition to one face of a fabric base, drawing said composition into depressions and openings in said fabric base without drawing said composition to the opposite side of said fabric, drying said coated fabric and thereafter working said fabric to render it sufficiently flexible. 45
13. A method of forming a coated fabric which comprises applying a coating to a fabric drawing said coating into the openings in said fabric while avoiding the impregnation of the threads of said fabric, drying said coating and working said coated fabric until sufficiently flexible. 40

In testimony whereof, I affix my signature.

RALPH S. ALLEN.